

March 6, 1928.

1,662,026

G. R. BROPHY

METALLIC GEAR AND METHOD OF MAKING THE SAME

Filed Sept. 2, 1925



Inventor:  
Gerald R. Brophy,  
by Alexander S. Gant,  
His Attorney

Patented Mar. 6, 1928.

1,662,026

# UNITED STATES PATENT OFFICE.

GERALD R. BROPHY, OF SCHENECTADY, NEW YORK, ASSIGNOR TO GENERAL ELECTRIC COMPANY, A CORPORATION OF NEW YORK.

## METALLIC GEAR AND METHOD OF MAKING THE SAME.

Application filed September 2, 1925. Serial No. 54,150.

The present invention relates to gears and has for its object to improve their construction, and also the method of making the same.

5 My improved gear is intended especially for use where the service or duty is especially severe, as for example, with electric railway motors, but it may advantageously be used for many other purposes.

10 Railway gears are commonly made of solid steel billets of circular cross-section, in which the fibers, by reason of the forming operations, extend lengthwise. These billets are afterwards cut into suitable lengths

15 to form blanks from which the gears are formed. The purpose of using round billets is to avoid waste of material and to decrease the cost of machine operations. These billets, however, due to the duty required of 20 the gears made therefrom, are relatively expensive.

As a result of the above-mentioned method of construction all or practically all of the fibers in the steel extend lengthwise of the 25 teeth and body whereas to obtain the greatest strength they should extend perpendicularly thereto.

To attain the desired relation of the fibers in the finished gear and also to lessen the 30 effect of flaws, I build up the blank out of steel laminations, which are punched to approximate size, using for the purpose sheet stock of say one-eighth inch in thickness, in which the fibers extend generally in the same 35 direction and in which flaws seldom occur. In other words, such stock possesses the important properties of being tough and uniform in texture. Ordinarily, the few flaws which occur in such sheets can readily be 40 detected but if not discovered by reason of being wholly between the side surfaces or for any other reason, no particular harm will be done because the defect is limited to a very small area and generally to a single 45 disk. The disks which form the blank may be smooth on the periphery but preferably they are provided with unfinished teeth formed to approximately the final shape and size of the finished teeth, allowing a sufficient 50 amount of material machining, so as to reduce the cost of the tooth cutting operation. Where gears of one or a few sizes are to be produced in quantities, the latter method of procedure is superior to the 55 former as will be evident. For my improved

gears, I use a low carbon sheet steel for subsequent carbonizing, or a medium carbon steel (40-50c), the cost of which per pound is only a fraction of what the billets cost. Having punched out the disks and removed 60 the burrs if any on the edges, a sufficient number are stacked to form a finished blank. In the stacking operation it is preferable to angularly displace the disks somewhat one with respect to the other so that the fibers 65 in the several disks will not all extend in the same direction but will be angularly displaced in the adjacent disks. No particular care need be observed in this respect, if the operators stacking the disks take them from 70 a pile of stock the resulting stack will generally be good enough.

The next step is to unite the disks one with the other. This is done by fusion of metal and for this purpose purified copper 75 is used, the fusion taking place in an electrically heated closed furnace in the presence of hydrogen or equivalent non-oxidizing gas. When in the furnace, the disks, to obtain the best results, should be retained 80 under pressure to prevent spaces being formed between them.

When a blank made in the manner set forth above is subsequently machined and polished it has the appearance of being made 85 of a single piece, and it is only by careful inspection that the joints between laminations can be detected. The copper used in fusing may be placed on top of the blank or around the periphery or it may be distributed both above and below the blank as well as around it, or very thin sheets placed between laminations. After the blank has been heated to a degree somewhat above the melting point of copper, the copper will flow 90 by capillary action into all of the joints between the disks and alloy to some extent with the adjacent surfaces of the steel disks. After the fusion takes place, the temperature is reduced to permit the copper to 95 harden after which the blank may be cooled in the open air or in a special cooler as desired. By actual tests it has been found that the joint between two pieces of steel united in the manner set forth is stronger 100 than the steel itself. This is probably due to the alloying of the steel with the copper. The disks or laminations may be weighted 105 while in the furnace to ensure good contact one with the other.

Another and successful way is to clamp the disks under heavy pressure and when in this condition to unite them by arc welding, the welds extending axially. Four such 5 welds would ordinarily be satisfactory but a greater or less number may be employed.

After the blank is removed from the furnace and has cooled the teeth are cut by the usual gear-cutting tools. Where the blank 10 has teeth formed approximately to size the tooth-cutting operation or finishing is much simplified and the rate of cutting or machining operation correspondingly increased. The gears may afterwards be case-hardened 15 by the usual methods. Blanks made in accordance herewith and afterwards properly machined and polished, show clearly uniform hardening of the steel surfaces. Railway motor pinions made in accordance with 20 my invention are now being used in daily service with successful results.

In the accompanying drawing which is 25 illustrative of my invention, Fig. 1 is an end view of a small gear or pinion; Fig. 2 is a longitudinal section of the same; and Fig. 3 is a view in side elevation of a blank 30 showing the temporary means employed to hold the laminations.

4 indicates the relatively thin disks which 35 are punched from sheets of low carbon steel. By preference the teeth 5 are approximately formed to shape and size in the punching operation. To reduce machine work each disk preferably has a central opening. 40 Where the bore of the finished gear is cylindrical the diameter of the openings will approximate the size of the finished bore but where the bore is to be slightly coned, as shown in Fig. 2, the diameter of the openings will approximate that of the small end 45 of the shaft.

In Fig. 2 the light parallel lines 6 indicate the copper-alloyed joints between the individual disks. In actual practice the joints 45 are very minute and on a well-polished surface are hardly noticeable. This is due to the fact that the spaces between the disks prior to the actual fusion are of a capillary nature and hence the amount of copper 50 which enters them is very small indeed.

One way to insure that the spaces between disks shall be of the desired character, the disks, after being properly stacked with the teeth thereon in register, is to subject the 55 stack to heavy endwise pressure, and while

so compressed to lightly weld them with an arc welder. Welds of this character are indicated at 7 in Fig. 3. The next step is to fuse the disks into a unitary structure and this is done in an electric furnace in an atmosphere of hydrogen or other non-oxidizing gas. The copper used for fusing can be applied to the blank in any well known way. 60

A gear to give the most satisfactory results in service should have a relatively soft 65 center with hardened teeth to reduce wear. To prevent the center from being hardened it is necessary to protect the same in the case-hardening operation. This may be done by any of the well known methods such as 70 copper plating.

What I claim as new and desire to secure by Letters Patent of the United States, is:—

1. A gear comprising laminations of sheet 75 steel, which laminations are united by fused copper.

2. A gear comprising laminations of sheet 80 steel in which the fibers thereof extend perpendicular to the axis, said laminations being united by fused copper.

3. A gear comprising steel laminations 85 which form the body and the teeth, said laminations being united by fused copper, the teeth being hardened.

4. A gear comprising laminations of sheet 90 steel in which the fibers thereof extend perpendicular to the axis, said laminations being united by fused copper and forming both the body and the teeth, the latter being case-hardened.

5. A gear comprising laminations of sheet 95 steel having a 40-50 carbon content in which the fibers thereof extend perpendicular to the axis, said laminations being united by fused copper and forming both the body and the teeth, the latter being hardened.

6. The method of making gears which comprises punching sheet steel to form disks of approximately the shape and size of the finished gear, assembling the disks in a stack 100 with the fibers of the steel extending perpendicular to the axis, holding the disks under pressure, uniting the disks by fused copper in a non-oxidizing atmosphere, finishing the teeth to exact size and finally 105 hardening the working surfaces of the teeth.

In witness whereof, I have hereunto set my hand this 1st day of September 1925.

G. R. BROPHY.